

## UNITED STATES PATENT OFFICE.

LUCIEN LIAIS, OF PARIS, FRANCE.

## METHOD OF MANUFACTURE OF AGGLOMERATED FUEL.

No Drawing. Application filed April 5, 1926, Serial No. 99,987, and in France April 30, 1925.

My invention relates to the manufacture of agglomerated fuel in all suitable forms whether in bricks or blocks, eggs perforated or plain, and in like forms, produced by the compression of dust or particles of fuels such as bituminous or anthracite coal, lignite, peat or the like, with the use of a binding material consisting of coal tar, bitumen or petroleum tar, or like substances.

10 In the known methods of manufacture, the binding material is added in the proper proportion to the powdered fuel, and the mixture is placed in a mixing machine which is heated by steam or by like means whereby 15 the binding substance—tar bitumen or the like—is melted. The paste formed by the machine is then brought to the agglomerating machine.

20 In the usual processes, the binding material represents 8-10 per cent, in order to obtain a cohesion varying from 60 to 80 per cent.

25 In the present invention I provide certain improvements whereby the usual manufacturing processes for agglomerated fuel will be made more economical, inasmuch as I can employ a given quality of fuel and binding material to attain the same degree of cohesion of the agglomerated material, with 30 the use of a less amount of binding substance, or only 5, 5-6 per cent, whereby the agglomerated products will be much reduced in cost, in view of the great expense for the binding material at present employed, and 35 chiefly such substances as coal or oil tar.

According to my invention, I add bicarbonate of soda to the binding material in the proper proportions, either in the form of crystals or as an aqueous solution, and due 40 to the resulting disengagement of carbonic acid in the presence of the tar or bitumen melted in the said mixing machine, there is obtained an improved distribution in the mass of the powdered fuel to be agglomerated, whereby the same degree of cohesion with a less amount of binding substance is afforded.

45 I dispose the bicarbonate of soda in the binding substance before placing the tar and the powdered fuel in the mixing machine, and I prefer to thus dispose it before the tar is combined with the fuel, and for instance it is placed in the endless screw feed-

ing conveyer for the tar, the proper quantity being poured by hand or by automatic means and in a continuous or intermittent manner into the said tar feeding device, according as the tar is supplied by the conveyer to the trough or belt which leads the fuel into the mixing machine.

55 By way of a comparative indication as concerns the known processes for the agglomeration of powdered fuel, such processes employ about 910 kgs. of powdered fuel and 90 kgs. of binding material to obtain 1000 kgs. of agglomerated products having 60-80 per cent cohesion.

60 Due to my said improvements, I am enabled to employ only 945 kgs. of powdered fuel and 55 kgs. of binding material to obtain 70 the same quantity of agglomerated products having substantially the same degree of cohesion, which represents an economy of about 35 kgs. of binding material per ton of agglomerated products, with a 75 very small expense for the bicarbonate of soda, which is used to the extent of only 1 kg. per ton of products.

Obviously, without departing from the principle of the invention, I may substitute 80 for the bicarbonate of soda any other suitable substance capable of causing a great disengagement of carbonic acid gas or like gas, in the aforesaid conditions.

What I claim is:

85 1. A fuel substance comprising, in combination, a pulverulent carbonaceous material, a viscous binder, and a sodium salt of carbonic acid.

2. A fuel substance comprising, in combination, coal dust, tar, and sodium bicarbonate.

90 3. The method of briquetting fuel which consists in pulverizing the fuel, mixing with a tar and sodium bicarbonate at an elevated 95 temperature.

4. The method of briquetting fuel which consists in heating a coal tar, causing to combine therewith sodium bicarbonate for the liberation of carbon dioxide, causing the 100 carbon dioxide to permeate the tar and convert it into a tar foam, pulverizing a fuel material, mixing the pulverized fuel with the foamed tar and forming the mixture into briquettes.

105 5. The fuel substance comprising, in com-

bination, a pulverized carbonaceous material, coal tar pitch, and sodium bicarbonate.

6. The fuel substance comprising in combination, a pulverulent carbonaceous material, a viscous binder, and an alkali metal salt of carbondioxide.

7. An article of manufacture comprising

briquettes containing powdered fuel, binder, and sodium bicarbonate, in the proportion of 944 parts of fuel, 55 parts of binder, and 10 one part of sodium bicarbonate.

In testimony whereof I affix my signature.

LUCIEN LIAIS.